

Jan. 5, 1932.

H. W. PORTH

1,839,498

DRY CELL

Filed May 21, 1929

Fig. 1.



Fig. 2.



INVENTOR  
*Henry W. Porth*

BY

Pennie, Davis, Marvin & Edwards  
ATTORNEYS

## UNITED STATES PATENT OFFICE

HENRY W. POETHE, OF MADISON, WISCONSIN, ASSIGNOR TO BURGESS BATTERY COMPANY, OF MADISON, WISCONSIN, A CORPORATION OF WISCONSIN

## DRY CELL

Application filed May 21, 1929. Serial No. 304,760.

This invention relates to an improved dry cell.

It is an object of this invention to improve the performance of a dry cell both on shelf and on discharge.

A dry cell of the Leclanché type may be made in several ways but usually has a gelatinous film or a paper pulp separator between the zinc or negative electrode and the depolarizing mix. The cells may be either of the round or flat types. Fig. 1 illustrates in cross section the round type of cell having a gelatinous electrolyte while Fig. 2 illustrates in cross section the round type with a paper pulp separator.

In a gelatinized paste cell a depolarizing mix 1 consisting of magazine dioxide, carbon or graphite, sal ammoniac and zinc chloride is molded around a central carbon electrode 2 which has a brass cap 3. The molded mix and carbon, usually called a core, may have an insulating bottom 4 attached to it and a bibulous wrapping of cheesecloth 5 is arranged around it. A gelatinous electrolyte 6 surrounds the core and forms a conducting path from the core to a zinc can or anode 7. A wax or pitch seal 8 rests on a washer 9 in the top of the can and the washer is spaced from the top of the core to form an expansion space 10.

In the paper pulp lined type of cell, Fig. 2, a zinc can 11 has a paper pulp lining 12. The depolarizing mix 13 is tamped in place around the carbon rod 14 which has a brass cap 15. Sand and sawdust 16 cover the top of the depolarizing mix. A wax or pitch seal 17 forms the cell closure.

Dry cells are used for a large variety of purposes. Under some conditions a cell may be discharged rapidly and under others it may be discharged slowly, either continuously or intermittently; the discharge period sometimes extending over a period of a year or more. The cell may be idle for a long period of time in the consumer's possession or it may be idle for a long period on a dealer's shelf before being sold and put into service.

It is very objectionable for a dry cell to deteriorate or lose its strength during these periods of idleness.

The dry cell industry has striven for years to overcome such objection and has met with varying degrees of success. It is the object of this invention to provide a dry cell which advances another step in the accomplishment of this purpose.

It has been known to the art for a long time that mercury or a mercury salt has a beneficial effect upon the life of a dry cell. The mercury amalgamates with the zinc and it apparently is this action which produces the beneficial effect. Likewise, chromic acid or a salt of chromic acid prolongs the shelf life as described in U. S. Patent No. 1,331,877, issued February 24, 1920. The CrO<sub>3</sub> radical seems to form a protective film on the zinc surface which prolongs the life of the cell when on open circuit.

Although both mercury and the CrO<sub>3</sub> radical produce beneficial effects separately I have found that by the combination of the two the effect is more than additive. I have found that a cell containing both of these ingredients shows a remarkably long life when put on light intermittent discharge. This type of discharge is the type encountered in the B and C circuits of radio apparatus.

I have not been able to determine the cause of the remarkable results obtained on light intermittent discharge but I have made observations which may give some clue to the explanation. If a mercury salt is introduced into the dry cell, preferably by introducing it into the gelatinous electrolyte containing zinc chloride, ammonium chloride, water and a gelatinized starch as exemplified by Hambuechen Patent No. 1,292,764, is issued January 28, 1919, but without the CrO<sub>3</sub> radical present, the zinc soon becomes darkened due to the amalgamation of the mercury with the zinc. If the chromic acid radical is introduced along with the mercury salt I have discovered that this amalgamation is prevented almost entirely except over long periods of time and on discharge. The zinc remains bright and maintains a clean surface in contact with the electrolyte.

A possible explanation is that a protective film is formed upon the zinc electrode by the chromate and this film prevents the mercury

from attacking the zinc rapidly thus slowing up the amalgamation. Another explanation is that the mercury may unite with the  $\text{CrO}_3$  radical to form mercuric chromate which is somewhat soluble in the electrolyte and gradually breaks down releasing mercury to effect the slow amalgamation of the zinc. However that may be, the explanation of the beneficial results obtained appears to lie in the keeping of the zinc surface clean and preventing its rapid amalgamation by the mercury.

I believe that the results obtained demonstrate that a slow amalgamation during the slow discharge of a cell is much to be preferred to the rapid amalgamation which is obtained when mercury is used in the absence of the  $\text{CrO}_3$  radical.

For the most successful attainment of the above described improved qualities in a dry cell, mercury should be present in the amount of from 0.00004 to 0.0006 grams and the  $\text{CrO}_3$  radical in the amount of from 0.00004 to 0.002 grams per square centimeter of zinc exposed to the electrolyte. I prefer to use mercury in the amount of 0.00008 to 0.0003 grams and the  $\text{CrO}_3$  radical in the amount of 0.0001 to 0.001 grams per square centimeter of zinc exposed to the electrolyte. I also prefer having  $\text{CrO}_3$  present in an amount equal to at least the chemical equivalent of the mercury in the cell.

Mercury may be successfully introduced in many forms, as metallic mercury or any salt of mercury. My preferred form is mercuric chloride. Likewise the  $\text{CrO}_3$  radical may be introduced in various forms, as chromic acid or any alkali or soluble salts of chromic acid. I prefer to use sodium dichromate.

The method of introducing the mercury and  $\text{CrO}_3$  radical should be designed to best meet the conditions. The mercury salt and the  $\text{CrO}_3$  radical may be added to the electrolyte at any time before gelatinization occurs in the amounts of about .01% to .2% of mercury salt calculated as metallic mercury and .01% to .5% of the  $\text{CrO}_3$  radical calculated as such. This will usually result in about the correct amount of mercury and  $\text{CrO}_3$  radical but these amounts must be kept within the limits based upon surface of zinc exposed to electrolyte as above set forth. Best results are obtained when the mercury is present in from .025% to .10% of the finished electrolyte and the  $\text{CrO}_3$  radical in from .025% to .25%.

In the paper pulp lined type of cell as illustrated by Fig. 2 the active depolarizing mix 13 usually contains the mixed chloride of ammonium and zinc in the desired amounts as is familiar to all who are skilled in the art. There are several satisfactory methods of introducing the mercury and  $\text{CrO}_3$  radical into this cell. Water or an

aqueous suspension of starch may be employed to moisten the paper pulp lining 12 prior to its insertion into the can 11. The mercury and  $\text{CrO}_3$  radical in the amounts hereinbefore specified may be introduced in the water or in this suspension. In both of the above described types of cells, the  $\text{CrO}_3$  radical in the form of a salt and mercury in the metallic form or as a salt can be conveniently incorporated in the active depolarizing mix. Other methods for introducing these materials will become apparent to those skilled in the art.

Although I prefer to introduce the  $\text{CrO}_3$  radical and mercury into the cell by dissolving salts of these two materials in the electrolyte or by introducing them into the mix or paper partition, as hereinbefore described, it is also possible to mix the mercury and  $\text{CrO}_3$  salts before introducing them into the cell thereby forming a mercury salt of chromic acid. It is possible to use this mercury salt of chromic acid in the same manner as the separate salts were used before they were combined. Throughout the specification and claims I do not wish to be restricted to adding the chromic acid radical and the mercury salt separately to the electrolyte but I also include the formation of a mercury salt of chromic acid prior to its addition to the cell.

This application is a continuation, in part, of my copending application, Serial No. 235,768, filed Nov. 26, 1927.

I claim:

1. In a dry cell comprising a zinc anode, a carbon cathode, a depolarizing mixture arranged between the anode and cathode, and a non-acid electrolyte; a mercury salt and  $\text{CrO}_3$  radical operatively associated with the electrolyte.

2. In a dry cell comprising a zinc anode, a carbon cathode, a depolarizing mixture arranged between the anode and cathode, and a non-acid electrolyte; mercuric chloride and a salt of  $\text{CrO}_3$  in the electrolyte.

3. In a dry cell comprising a zinc anode, a carbon cathode, a depolarizing mixture arranged between the anode and cathode, and a non-acid electrolyte; mercuric chloride and sodium dichromate in the electrolyte.

4. In a dry cell comprising a zinc anode, a carbon cathode, a depolarizing mixture arranged between the anode and cathode, and a non-acid electrolyte; a mercury salt and at least enough salt of chromic acid in the electrolyte to retard amalgamation of the zinc can by the mercury.

5. In a dry cell comprising a zinc anode, a carbon cathode, a depolarizing mixture arranged between the anode and cathode, and a non-acid electrolyte; mercuric chloride and at least enough dichromate in the electrolyte to retard amalgamation of the zinc can by the mercury.

6. A dry cell having a zinc anode and a non-acid electrolyte containing a mercury salt and  $\text{CrO}_3$  in the electrolyte, said  $\text{CrO}_3$  being present in an amount equal to at least 5 the chemical equivalent of said mercury.

7. A dry cell having a zinc anode and containing in its electrolyte substantially .00004 to .0006 grams of mercury in the form of mercury salt per square centimeter of zinc 10 exposed to said electrolyte and substantially .00004 to .002 grams of the  $\text{CrO}_3$  radical per square centimeter of zinc exposed to said electrolyte.

8. A dry cell having a zinc anode and containing in its electrolyte substantially .00008 to .0003 grams of mercury in the form of a mercury salt per square centimeter of zinc exposed to said electrolyte and substantially .0001 to .001 grams of the  $\text{CrO}_3$  radical per 20 square centimeter of zinc exposed to said electrolyte.

9. An electrolyte paste for a dry cell containing from substantially .01% to .2% mercury in the form of a mercury salt and from 25 substantially .01% to .5% of the  $\text{CrO}_3$  radical.

10. An electrolyte paste for a dry cell containing from substantially .025% to .1% mercury in the form of a mercury salt and from 30 substantially .025% to .25% of the  $\text{CrO}_3$  radical.

In testimony whereof I affix my signature.  
HENRY W. PORTH.

35

40

45

50

55

60